

## UNITED STATES PATENT OFFICE

2,282,351

## ELECTROLYTE FOR AND METHOD OF POLISHING METAL SURFACES ANODICALLY

Charles L. Faust, Columbus, Ohio, assignor to Battelle Memorial Institute, Columbus, Ohio, a corporation of Ohio

No Drawing. Application October 5, 1940,  
Serial No. 359,936

8 Claims. (Cl. 204—140)

This invention relates to an electrolyte for and to a method of finishing metal surfaces anodically. More particularly the invention relates to the anodic treatment of metals in an aqueous electrolyte containing arsenic acid or the equivalent arsenate radicals having a total acid concentration, furnished either by arsenic acid itself, or by an admixture of arsenic acid with sulfuric, phosphoric, chromic or other suitable acid, of from 50% to 95% by weight. By the selection of an electrolyte composition containing arsenic acid and one or more of the other acids named, within the limits of total acid concentration specified, it is possible to impart to the surface of a metal, when treated as an anode therein, a lustrous, mirror-like polish.

This constitutes a continuation-in-part of my application of the same title, Serial No. 290,787, filed August 18, 1939.

It has heretofore been proposed to use various compositions of electrolyte for the anodic treatment of metal. In some cases the object has been to clean the metal surface by the etching action of the electrolyte, while in other cases the etching effect has been reduced to a minimum and the object has been to produce a lustrous image reflected surface. The anodic treatment of aluminum has a somewhat separate status, since there the purpose has been not only to provide a lustrous surface but also to form thereon a dense, adherent layer of aluminum oxide as a protection therefor against corrosion and wear.

I have now found that an electrolyte containing arsenic acid, or an equivalent arsenate radical, in an aqueous acid solution of sufficient total acid concentration can be satisfactorily employed in the anodic treatment of various metals and alloys to impart to the surfaces thereof the desired type of finish. In the preferred embodiment of my invention, which will be described more specifically hereinafter, such an electrolyte is employed for imparting a lustrous, mirror-like surface, but its use is not limited to that purpose alone.

It is therefore an important object of my invention to provide an electrolytic solution containing arsenic acid, or arsenate radicals, and having a relatively high total acid concentration for use in the anodic treatment of metals generally to impart thereto a desirable surface finish.

It is a further important object of my invention to provide an electrolyte for and a method of anodically treating metals and alloys to produce thereon surfaces that are highly lustrous and free from the scratches and "piled" layers char-

acteristics of mechanically polished metal surfaces.

It is a further important object of this invention to provide a method for the anodic polishing of metals by making the metal to be polished the anode in an electrolyte of relatively high acid concentration containing arsenic acid, or equivalent arsenate radicals, and one or more mineral acids.

10 Other and further important objects of this invention will become apparent from the following description and appended claims.

A method to which this invention pertains involves making the metals to be treated an anode in an electrolytic bath of suitable composition and passing a current therethrough of sufficient density and for a sufficient length of time to produce the desired type of surface finish, which, more specifically may be a highly lustrous or mirror-like polish.

The electrolyte that I have found to possess the most general applicability comprises an aqueous solution of arsenic acid, either by itself or in admixture with sulfuric acid, phosphoric acid, or chromic acid, or two or more of such acids. The term arsenic acid is intended to include any of the various forms of arsenic acid, such as ortho, meta and pyro, that may be used as such in making up the aqueous electrolyte or that may be formed in the electrolyte as the result of the action of the strong mineral acid or acids, upon the particular arsenate compound added. For satisfactory results, the concentration of arsenic acid ( $H_3AsO_4$ ) should be between 5 and 93% by weight of the solution, and if used alone, the arsenic acid concentration should be at least 50% by weight of the solution. It is generally preferable to include one or more of the other mineral acids in the electrolyte, and, in that case, the combined acid concentration should be between 50 and 95% by weight of the solution. The mineral acids preferred for admixture with the arsenic acids are sulfuric acid within the range of from 0 to 85%, phosphoric acid within the range of 0 and 85%, and chromic anhydride ( $CrO_3$ ) within the range of from 0 to saturation. If it is desired to obtain the highest degree of polish of surfaces of the metals or alloys undergoing treatment, the minimum combined acid concentration should be not less than 60% by weight. Aside from such metallic salts as may be present in the solution due to anodic dissolution of the metal undergoing treatment, the balance of the electrolytic solution will be largely water. There will thus be a minimum of 5% and a maximum of

50% of water in the electrolyte of my invention.

While it is possible to produce desirable surface effect with mixtures of arsenic and other acids containing as much as 50% water, I prefer to keep the water content of the electrolyte relatively low, since I have found, in general, the bath containing the lower proportions of water may be operated at lower current densities, and therefore at a lower cost for electrical current.

It will be understood, of course, that during the operation of an electrolyte such as described, there will be a gradual building up of the content of metal salts formed by dissolution of the metal undergoing anodic treatment. There also may be some change in the water content due to loss of water by evaporation or as a result of electrolytic decomposition or due to gain of water by condensation or collection of moisture from the air. The composition of the electrolyte should, however, be kept within the foregoing limits as to total acid concentration and water content if satisfactory operating conditions are to be maintained.

The following will serve to illustrate preferred compositions of my electrolyte:

*Example 1*

For use in the electropolishing of stainless steel, rustless iron, nickel and nickel alloy, I have found that any one of the following baths is entirely satisfactory:

|                             | Bath    |         |         |
|-----------------------------|---------|---------|---------|
|                             | No. 1   | No. 2   | No. 3   |
|                             | Percent | Percent | Percent |
| Sulphuric acid              | 36      | 25      | 10      |
| Arsenic acid ( $H_3AsO_4$ ) | 47      | 69      | 77      |
| Water                       | 17      | 6       | 13      |
|                             |         | 40      |         |

With the foregoing compositions of electrolyte, excellent polishes have been obtained on 18-8, 25-12 chromium-nickel stainless steels, plain carbon steels, copper, brass, nickel, and nickel alloys, such as Monel metal, and Chromel, operating the bath at a temperature of about 60° C. and employing an anode current density of from 50 to 100 amperes per square foot and upwards.

*Example 2*

The following bath was effective in the electro-polishing of copper where the metal was made an anode with a current density of 385 amperes per square foot and a temperature of 55° C. for fifteen minutes:

|                          | Per cent |
|--------------------------|----------|
| Arsenic acid             | 84       |
| Chromic acid ( $CrO_3$ ) | 10       |
| Water                    | 6        |
|                          | 60       |

This same bath was also effective in polishing zinc at a current density of 340 amperes per square foot at a temperature of 63° C. for eight minutes. Alloys of zinc and copper, stainless steel and nickel alloys could also be polished in this bath under comparable conditions.

*Example 3*

The following bath was effective in the polishing of 18-8 type of stainless steel and copper:

|                      | Per cent |
|----------------------|----------|
| Arsenic acid         | 15       |
| Orthophosphoric acid | 60       |
| Water                | 25       |
|                      | 75       |

This bath produced a mirror finish on stainless steel at current densities of 250 amps./sq. ft. and a temperature of around 50 to 70° C., when the metal was treated anodically for 40 minutes. A mirror finish was also produced on copper at a current density of 500 amps./sq. ft. operated for 23 minutes.

*Example 4*

The following bath was found to be effective for polishing brass when the brass was treated anodically for thirty minutes at a current density of 500 amps./sq. ft.

|                      | Per cent |
|----------------------|----------|
| Arsenic acid         | 15       |
| Orthophosphoric acid | 55       |
| Chromic acid         | 3        |
| Water                | 27       |

*Example 5*

A desirable finish can be produced on aluminum by treating the aluminum anodically in a bath of the following composition:

|                          | Per cent |
|--------------------------|----------|
| Arsenic acid             | 25       |
| Sulfuric acid            | 15       |
| Orthophosphoric acid     | 35       |
| Chromic acid ( $CrO_3$ ) | 10       |
| Water                    | 15       |

In the case of aluminum, the current density is limited by the anodic film which forms.

In general, anode current densities varying from 50 to 1000 amps./sq. ft. may be employed, depending upon the type of surface treatment that is desired, the type of metal or alloy undergoing treatment and the composition of the electrolyte. Higher current densities than indicated by the foregoing range may also be employed, but in that case the higher current cost offsets the saving in time. The length of time to effect the desired results depends upon the magnitude of the current density employed, and to some extent upon the particular metal or alloy undergoing treatment and the character of the metal surfaces initially. Rough surfaces, of course, require a longer time to polish than relatively smooth ones.

As illustrative of the length of time required to effect a high degree of electropolish, from 5 to 90 minutes is usually found sufficient. The temperature at which the anodic treatment is carried out, while preferably between 50 and 75° C., may be varied from around room temperature to temperatures only slightly under the boiling point of water.

From the foregoing description of my invention, it is apparent that I have provided a novel composition of electrolyte for use in the anodic treatment of metals.

While an aqueous solution of arsenic acid alone is satisfactory for polishing some metals and alloys, as for instance 18-8 stainless steel, it is preferable to use another acid with it, such as chromic anhydride, sulfuric acid, or ortho-phosphoric acid. Where a mixture of only two acids is used, such as arsenic-chromic, arsenic-sulfuric, or arsenic-phosphoric, the limits for the arsenic acid are as above stated, viz. from 5 to 93%; the limits for chromic anhydride from 0.1% to saturation; the limits for sulfuric acid from 5 to 85%; and the limits for ortho-phosphoric acid from 5 to 85%. The combined acid concentration in any case should be between 50 and 95%.

It will, of course, be understood that various details of the process may be varied through a

wide range without departing from the principles of this invention and it is, therefore, not the purpose to limit the patent granted hereon otherwise than necessitated by the scope of the appended claims.

I claim as my invention:

1. An electrolyte for use in the anodic polishing of metals, comprising an aqueous solution of about 84% arsenic acid, 10% chromic anhydride and 6% water by weight.

2. An electrolyte for use in the anodic polishing of metals, comprising an aqueous solution of about 15% arsenic acid, 3% chromic acid, 55% orthophosphoric acid, and 27% water by weight.

3. An electrolyte for use in the anodic polishing of metals, comprising an aqueous solution of about 25% arsenic acid, 15% sulfuric acid, 35% orthophosphoric acid, 10% chromic anhydride and 15% water, by weight.

4. The method of electropolishing metals, which comprises making a metal the anode in an electrolyte comprising about 84% of arsenic acid, 10% of chromic acid and 6% of water, by weight, and passing a current therethrough of sufficient density and for a sufficient length of time to effect a polish on said metal surface.

5. The method of electropolishing metals, which comprises making a metal the anode in an electrolyte comprising about 15% of arsenic acid, 3% of chromic acid, 55% of orthophosphoric acid and 27% of water, by weight, and passing a current therethrough of sufficient density and for a sufficient length of time to effect a polish on said metal surface.

6. The method of electropolishing metals, which comprises making a metal the anode in an electrolyte comprising about 25% of arsenic acid, 15% of sulfuric acid, 35% of orthophosphoric acid, 10% of chromic anhydride and 15% of water, by weight, and passing a current therethrough of sufficient density and for a sufficient length of time to effect a polish on said metal surface.

10 7. An electrolyte for use in the anodic polishing of metals comprising an aqueous solution of from 5 to 93% of arsenic acid, from 0 to 85% of sulfuric acid and a significant amount of an acid selected from the group consisting of phosphoric acid and chromic acid and mixtures thereof, said solution having a combined acid concentration of at least 50% by weight, the balance being largely water.

15 8. The method of anodically polishing metals, which comprises making a metal the anode in an aqueous acid electrolyte comprising from 5 to 93% arsenic acid, from 0 to 85% of sulfuric acid and a significant amount of an acid selected from the group consisting of phosphoric acid and chromic acid and mixtures thereof, said electrolyte having a combined acid concentration of at least 50% by weight, the balance being largely water and passing an electric current therethrough of a sufficient density and for a sufficient period of time to effect the desired polish.

CHARLES L. FAUST.